

No. 882,990.

PATENTED MAR. 24, 1908.

L. E. BARRINGER.  
RESISTANCE UNIT.  
APPLICATION FILED SEPT. 30, 1907.

Fig.1.



Fig.2.



Witnesses

J. Earl Ryan  
J. Ellis Allen.

Inventor

Lawrence E. Barringer  
by *Alfred B. Davis*  
Atty.

# UNITED STATES PATENT OFFICE.

LAWRENCE E. BARRINGER, OF SCHENECTADY, NEW YORK, ASSIGNOR TO GENERAL ELECTRIC COMPANY, A CORPORATION OF NEW YORK.

## RESISTANCE-UNIT.

No. 882,990.

Specification of Letters Patent. Patented March 24, 1908.

Application filed September 30, 1907. Serial No. 395,130.

To all whom it may concern:

Be it known that I, LAWRENCE E. BARRINGER, a citizen of the United States, residing at Schenectady, county of Schenectady, 5 State of New York, have invented certain new and useful Improvements in Resistance-Units, of which the following is a specification.

My invention relates to a new combination of material for use in the production of a resistance stick or unit. This new combination of material produces results not heretofore attained with resistance sticks, and renders possible a wider application of said 15 sticks, as will be further described.

The accompanying sketch shows an application of these resistance units or members in lightning arresters, but their use may be extended to rheostats, car heaters, fan 20 motors resistances, and so forth, and in fact, to any electrical use where a uniform resistance is required.

Figure 1 is a front view of a well-known form of lightning arrester, and Fig. 2 is a side 25 view of the same.

The non-inductive resistance 1 and the metal cylinders 2, 3 of this arrester form part of a grounded circuit. A current of very high potential such as a lightning discharge, 30 will jump the gap between 2 and 3 and be grounded. This form of lightning arrester is well-known and hence will require no further description here. For the non-inductive resistance 1, I propose to use the resist- 35 ance member or unit hereinafter described.

As a novel ingredient of my resistance unit I use a material well known to the trade as "alundum". Alundum is a very hard, crystalline material made from bauxite, an amorphous hydrate of aluminium, by a process of 40 purification and electric furnace treatment. The material resulting from this treatment is essentially a fused alumina, of a high degree of purity and uniformity. It is a sort of 45 artificial corundum composition, as it corresponds in general to the chemical formula  $Al_2O_3$ . The alundum is mixed in various proportions with clay and graphite according to the properties desired in the finished 50 product. I have used the following proportions in preparing my resistance unit. 20 parts alundum, 20 parts fire clay (with which may be mixed, if desired, suitable amounts of feldspar and flint); 1½ to 2½ 55 parts of graphite. As the graphite is added

to give the stick conductivity, its proportion is variable. These materials are thoroughly mixed, preferably wet, squirted into shape, dried and baked at a temperature of 1100 degrees to 1300 degrees. The sticks may be 60 enameled with any known enamel to keep out moisture. Contact surfaces may be made at each end in any known way, such as carbonizing the ends, copper-plating them, shrinking on them metal caps, or the like. 65 Each ingredient mentioned above has a positive and regular effect on the ultimate product. The alundum gives the unexpectedly beneficial results hereinafter set forth. The graphite serves to give the requisite conductivity, and the clay base serves as a binding material to form a strong, compact rod or stick. As a clay binder or base, I prefer to employ a high grade fire clay. If a more 70 vitreous mass should be desired, an admixture of feldspar and flint may be made, as above mentioned.

I am aware that a combination of carborundum, clay base and graphite has been used in the production of a resistance stick but the 80 use of this material was accompanied with certain disadvantages. The resistance of a rod containing this material changes in an irregular manner during heating. The resistance is generally higher on cooling than 85 originally, sometimes lower, and only rarely does it approximate the original resistance. This fact alone barred out the use of these resistances in rheostats and other applica- 90 tions.

When alundum is employed instead of carborundum, I find that the resistance of the rods remains constant after heating. I consider this difference of behavior a most important one. While I do not wish to be limited by any particular theory I believe the behavior of carborundum rods may be attributed to the fact that the expansion and contraction of these rods in heating and cooling brings about a readjustment of the particles and a change in the contact of the conducting particles throughout the mass. As the coefficient of expansion of alundum is almost zero, these readjustments may not occur when this material is heated and cooled. Furthermore, it was found that the conductivity of the raw carborundum varied greatly. Hence, in order to make a rod of a given resistance, it was first necessary to determine 100 the conductivity of the carborundum by pre- 105 110

liminary experiments. This being determined, more or less graphite was added in the manufacture of the rod, according to the determined conductivity of the carborundum. This consumed time and involved expense.

With alundum we have a material whose conductivity is constant, that is, it is practically zero. Therefore in order to produce a given conductivity in the finished rod, a certain definite amount of graphite as an ingredient is added without the necessity for previous analysis.

A further advantage in the use of alundum instead of carborundum as an ingredient lies in the fact that the finished alundum sticks are less liable to crack and burst when heated to a high temperature. As is well known, the carborundum sticks crack and burst on heating to a high temperature.

In addition to the desirable qualities set forth, I find the alundum resistance sticks are tougher and stronger than the sticks made with carborundum. In the carborundum stick the clay base was practically the only source of strength, therefore, the prop-

erty possessed by alundum of adding an element of strength is a most desirable one.

What I claim as new and desire to secure by Letters Patent of the United States, is,

1. A resistance member consisting of alundum, graphite and fire clay.

2. A resistance member consisting of fused alumina, refractory conducting material, and a suitable binder.

3. A resistance member consisting of a mixture of alundum, graphite and clay.

4. A resistance member consisting of 20 parts of alundum, 20 parts of clay base, and  $1\frac{1}{2}$  to  $2\frac{1}{2}$  parts of graphite.

5. The combination of a resistance member consisting of alundum, graphite, and clay, an enamel upon the surface of said member, and means for making electrical contacts with the ends of said rods.

In witness whereof I have hereunto set my hand this 28th day of September, 1907:

LAWRENCE E. BARRINGER.

Witnesses:

BENJAMIN B. HULL,  
HELEN ORFORD.